

# UNITED STATES PATENT OFFICE.

LUDWIG VIRNEISEL, OF MANNHEIM, BADEN, GERMANY.

## METHOD OF MANUFACTURING HYDRATED GRAPE-SUGAR.

SPECIFICATION forming part of Letters Patent No. 310,339, dated January 6, 1885.

Application filed August 31, 1882. (No specimens.)

*To all whom it may concern:*

Be it known that I, LUDWIG VIRNEISEL, of Mannheim, Baden, Germany, have invented certain new and useful Improvements 5 in the Manufacture of Grape-Sugar, of which the following is a specification.

This invention relates to an improved method of manufacturing hydrated grape-sugar without the employment of alcohol or similar 10 separating agents; and the invention consists in making hydrated grape-sugar by first forming a magma of crystals of grape-sugar from a starch-glucose solution of a density of 25° to 30° saccharometer, then mixing the magma 15 with a thin colorless juice of grape-sugar and draining or washing off the syrup from the crystals, and finally drying the crystals at ordinary temperature.

In carrying out my invention a solution of 20 grape-sugar (starch-glucose) of a density of twenty-five to thirty saccharometer degrees is allowed to crystallize at ordinary temperature. The co-efficient of purity of this solution should not be below 95—that is to say, the glucose solution should contain in one hundred parts not 25 more than five parts which are not dextrose. The magma of crystals so formed is mixed at ordinary temperature, as rapidly and intimately as possible, with one-half to an equal 30 volume of a thin colorless juice of grape-sugar of 20° saccharometer scale in a macerator, such as are employed in beet-sugar factories. The resulting thin starch-glucose mash is transferred to a suction apparatus, and the 35 grape-sugar drained from the juice. This draining or washing operation with thin saccharine juice is repeated twice or three times, until pure white crystals of sugar are obtained, which are dried at ordinary temperature, 40 by means of a current of air. By thus forming first a magma of grape-sugar crystals, mixing them with thin juice or liquor by mechanical means, and separating then the uncry stallizable substances—such as syrup or 45 molasses—from the crystals by a suction apparatus, and then producing the complete removal of the uncry stallizable or unfermentable substances from the crystals by repeatedly washing or draining them by means of a 50 thin colorless juice at ordinary temperature, the use of alcohol or similar separating agents

which have heretofore been employed in the production of hydrated grape-sugar is dispensed with and a pure white grape-sugar monohydrate obtained, which contains from 55 eighty-nine to ninety-one per cent. of dextrose and from eleven to nine per cent. of water, and which, in contradistinction to the ordinary glucose of commerce, does not polarize to the right after fermentation.

I am aware that impurities have been removed from raw sugar by first mixing the same with a sugar syrup or liquor, and then washing the so-prepared raw sugar in a centrifugal machine.

I am also aware that refined cane-sugar has been mixed with grape-sugar by first draining the sugar magmas of their contained syrups, and then washing the drained sugar by a suitable washing-liquor, and finally charging the 70 drained and washed sugars with a solution containing grape-sugar. I, therefore, do not claim the processes referred to. The difference between these processes and my method consists, essentially, in forming, first, a magma 75 of crystals of grape-sugar hydrate from a starch-glucose solution of a determined density and purity, and then washing and draining the same until the pure crystals of hydrated grape-sugar are obtained.

Having thus described my invention, I claim as new and desire to secure by Letters Patent—

The process herein described of making hydrated grape-sugar, which consists, first, in forming a magma of crystals of grape-sugar hydrate from a starch-glucose solution of twenty-five to thirty saccharometer degrees, and of a co-efficient of purity of 95; secondly, mixing the magma thoroughly with a thin colorless juice of grape-sugar; thirdly, draining or washing off the syrup from the crystals and repeating the washing operation until the uncry stallizable or unfermentable substances are entirely separated from the crystals of hydrated grape-sugar, substantially as specified.

In testimony that I claim the foregoing as my invention I have signed my name in presence of two subscribing witnesses.

LUDWIG VIRNEISEL.

Witnesses:

MARTIN SAENGER,  
G. FRIED. GRÜN.